# EUROPEAN PATENT SPECIFICATION

(11) **EP 0 362 661 B1**
(45) Date of publication and mention of the grant of the patent: **08.03.1995**
(21) Application number: 89117666.1
(22) Date of filing: 25.09.1989
(51) Int. Cl.: C22C 19/05, C22F 1/10

(54) **Cast columnar grain hollow nickel base alloy article and alloy and heat treatment for making**
Gegossenes aus stengelförmigen Kristallen bestehendes hohles Werkstück auf Nickel basierender Legierung sowie die Legierung und Wärmebehandlung für dessen Herstellung
Pièce creuse en alliage à base de nickel coulé comportant une structure de grains colonaire, alliage et procédé de sa fabrication

(30) Priority: 03.10.1988 US 253109
(43) Date of publication of application: 11.04.1990
(73) Proprietor: GENERAL ELECTRIC COMPANY, Schenectady New York 12305 (US)
(72) Inventor: Ross, Earl Warren, Cincinnati Ohio 45229 (US); O'Hara, Kevin Swayne, Boxford Massachussetts 01921 (US)
(74) Representative: Pratt, Richard Wilson

(56) References cited:
- EP-A- 0 032 812
- EP-A- 0 155 827
- EP-A- 0 194 925
- EP-A- 0 246 082
- FR-A- 2 243 270
- FR-A- 2 374 427
- FR-A- 2 406 001

## Description

This invention relates to cast directionally solidified columnar grain nickel base alloy articles and, more particularly, to such an article of outstanding elevated temperature surface stability as represented by oxidation resistance, particularly in thin walled hollow articles, and to the alloy and neat treatment for making such article.

### BACKGROUND OF THE INVENTION

A significant amount of the published and well known casting technology relating to high temperature operating articles, for example turbine blades for gas turbine engines, has centered about improvement of certain properties through elimination of some or all of the grain boundaries in the final article's microstructure. In general, such structures have been generated by the well known precision casting techniques of solidifying a molten metal directionally (directional solidification) to cause the solidifying crystals or grains to be elongated. If only one grain is allowed to grow in the article during solidification, for example, through choking out others or using a seed crystal, an article of a single crystal and substantially no grain boundaries results. However, if multiple grains are allowed to solidify at an area of a casting mold and allowed to grow generally in a single direction in which heat is withdrawn from molten metal in a casting mold, multiple elongated or columnar grains exist in the solidified casting. Such a structure sometimes herein is called "DS multigrain" in connection with a cast article. The direction of elongation is called the longitudinal direction; the direction generally normal to the longitudinal direction is called the transverse direction.

Because the grain boundaries in such an article are substantially all longitudinal grain boundaries, it is important in an article casting that longitudinal mechanical properties, such as stress rupture life and ductility, be very good, along with good transverse mechanical properties and good alloy surface stability. With this property balance in the article, the article alloy must be capable of being cast and directionally solidified in complex shapes and generally with complex internal cavities and relatively thin walls without cracking. So called "thin-wall" hollow castings have presented difficult quality problems to article casters using the well known "lost wax" type of precision casting methods with alloys designed for improved properties: though the alloy properties are good and within desired limits, thin wall castings, for example with a wall less than about 0.889mm (0.035 inch) thick, generally cracked during multicolumnar grain directional solidification.

Briefly, in one aspect, the present invention provides a nickel base superalloy consisting of in weight percent 0.12% carbon, 1.5% hafnium, 12% cobalt, 6.35% tantalum, 6.8% chromium, 1.5% molybdenum, 4.9% tungsten, 6.15% aluminum, 2.8% rhenium, 0.015% boron, the substantial absence of zirconium, the substantial absence of titanium, the substantial absence of vanadium and the balance of nickel and incidental impurities.

Articles may be formed from the above alloy and are characterized by outstanding elevated temperature surface stability for a directionally solidified article, resulting from an alloy specification enhanced, in one form, by heat treatment and by an improved combination and balance between longitudinal and transverse stress rupture properties. In one form, the article has at least one internal cavity and includes an integral cast wall substantially free of a major crack, the wall having a thickness of less than about 0.889mm (0.035 inch).

In respect of the alloy of the present invention, a particular combination of the elemental addition of C, Hf, Co and Ta, and the intentional limitation of the elements V, Zr and Ti, provides outstanding elevated temperature oxidation resistance, good castability, and resistance to grain boundary and fatigue cracking in a Ni base alloy which also includes Cr, Mo, W, Al, Re and B.

Another aspect of the present invention associated with such alloy is a heat treatment involved in the method for making the article. Such heat treatment comprises a combination of at least three progressive heating steps including a solutioning step, a preliminary, first aging step and a second aging step, to improve stress rupture properties of the article.

Thus the present invention also provides a method of heat treating a cast nickel base alloy article made of an alloy consisting of, in weight percent, 0.1-0.15 C, 0.3-2 Hf, 11-14 Co, 5-9 Ta, less than 0.05 Zr, no more than 1 of V, no more than 1 of Ti, 5-10 Cr, 0.5-3 Mo, 4-7 W, 5-7 Al, 1.5-4 Re, 0.005-0.03 B, up to 1.5 Nb, up to 0.5 Y and the balance Ni and incidental impurities comprising the steps of :
(a) heating at a solutioning temperature in a non-oxidizing atmosphere for a time sufficient to solution at least 90% of the gamma-gamma prime eutectic and coarse secondary gamma prime and so that there is no more than about 4% incipient melting, and then cooling in the atmosphere to a temperature in the range of 1107-1135°C (2025°-2075°F);
(b) heating at a first aging temperature in the range of 1107-1135°C (2025°-2075°F) in a non-oxidizing atmosphere for about 1-10 hours and then cooling in the atmosphere to a temperature in the range of 1066-1093°C (1950°-2000°F); and
(c) heating at a second aging temperature lower than the first aging temperature in the range of 1066-1093°C (1950°-2000°F) for 4-12 hours.

Preferably the solutioning temperature is in the range of 1246-1293°C (2275-2360°F) and the heating time is at least about 30 minutes.

### BRIEF DESCRIPTION OF THE DRAWING

The drawing is a graphical comparison of oxidation resistance of the alloy associated with the present invention with other alloys.

### DESCRIPTION OF THE PREFERRED EMBODIMENTS

The nickel base alloy of the present invention is particularly characterized by the relatively high C content in combination with a relatively large amount of Hf and additions of Co and Ta. This, along with the intentional control and limitation of the elements V, Zr and Ti, enabled the total alloy to have, for a DS structure, outstanding oxidation resistance and the good DS castability and resistance to grain boundary and fatigue cracking to the point at which thin walls of less than 0.889mm (0.035 inch) can be DS cast with elongated grains substantially crack free. Other elements in the alloy, contributing to its unique mechanical properties and surface stability, in a nickel base, are Cr, Mo, W, Al, Re and B. The resultant article, with an unusual, unique combination of mechanical properties and surface stability, is particularly useful in making hollow, air cooled, high temperature operating components such as blading members (blades and vanes) of the type used in the strenuous environment of the turbine section of gas turbine engines. In rotating turbine blades which are subject to high stress as well as high temperature oxidation and hot corrosion, the crack free condition of thin walls associated with internal cooling passages, is essential to safe, efficient engine operation.

A measure of the castability and crack resistance of high temperature directionally solidified columnar grained nickel base superalloys is the castability test and rating scale reported in U.S. Patent 4,169,742 Wukusick et al, issued October 2, 1979, beginning in column 2 at line 41 and continuing into column 3. The rating is repeated here in Table I.

**TABLE I**

| CASTABILITY RATINGS | |
|---|---|
| A | No cracks |
| B | Minor crack at tip, less than 1.27cm (1/2") long or in starter zone |
| C | One major crack, greater than 1.27cm (1/2") long |
| D | Two or three cracks |
| E | Several cracks, more than 3 and less than 8 |
| F | Many cracks - most grain boundaries |

A selection of nickel base superalloys sometimes used or designed for use in gas turbine engine turbine components is presented in the following Table II along with a form of the particular alloy associated with the present invention. The alloy identified as Rene' N5, designed for use in making single crystal alloy articles, is described in US-A-5100484 and GB-A-2235697; the alloy identified as Rene' 150, designed for use as a DS columnar grain article, is described in the U.S. Patent 4,169,742. Also included in Table II are the castability ratings of such alloys.

An evaluation of varying Hf, Co and B in the alloy identified in Table II as Rene' N5 was conducted to improve castability. Results of such evaluation are shown in Table III.

The data of Table III show primarily the benefit and criticality of including Co at a level greater than 7.5 wt% (for example about 10 wt %) up to about 12 wt%, in combination with Hf in the range of about 0.3 - 1.6 wt%. However, even with such improved castability, the alloy modification of Rene' N5 alloy had reduced longitudinal stress rupture strength due to dilution of the hardening elements from the addition of more Co to the Rene' N5 alloy base chemistry of Table II above, at a C level of about 0.05 wt%. With the nominal 3% additional Co to the Rene' N5 Alloy composition (to make it a total of 10.5% Co) and nominally 1% Hf, longitudinal stress rupture life was about 65% of Rene' N5 alloy; with nominally 4.5% additional Co (to make it a total of 12% Co) and at 0.5% Hf, longitudinal stress rupture life was 30% of Rene' N5 Alloy. This is indicative of one critical balance of elements used in the method of the present invention, with an alloy composition including C in the range of 0.1 - 0.15 wt% along with Co in the range of 11-14 wt% and 0.3-2 wt% Hf.

In respect to the balance between castability, and grain boundary and fatigue cracking, it has been recognized that too little Co results in loss of castability and grain boundary strengthening, whereas above about 14 wt% Co can dilute the effect of certain alloy strengthening elements. The element Hf, if too low, such as below about 0.3 wt%, increases the tendency toward grain boundary cracking in DS casting and in use; and if too high, such as above 2 wt%, Hf can result in problems relating to casting reactivity and incipient melting during heat treatment. Too much Ta and Al can affect castability by being too strong and can cause grain boundary cracking. Also it can form Topologically Close Packed (TCP) phases. Therefore, the Ta content is maintained preferably in the range of 6-7 wt% and the Al preferably is 5.5 - 6.5 wt% in the practice of this invention. As is known in the art, small amounts of Nb may be substituted for Ta.

In the evaluation of some of the alloys of Table II, it was recognized that vanadium can detract from the surface stability, i.e., hot corrosion and oxidation resistance; Zr can increase crackability; and Ti can seriously reduce oxidation resistance. Therefore, these elements have been controlled and limited to the ranges in weight percent of less than 1 V, 0.05 Zr and 1.5 Ti, preferably less than 0.1V, 0.03 Zr and 0.02 Ti. While yttrium is helpful in improving oxidation resistance, it can cause grain boundary weakening; thus, it is limited to amounts less than 0.1% in the alloys of the invention. Cr is included primarily for its contribution to oxidation and hot corrosion resistance; Mo, W and Re primarily for matrix strengthening and B to enhance grain boundary strength.

Although the castability of such alloys as Rene' 150 were very good and within the acceptable range for thin wall castings, their surface stabilities were unacceptable for certain high temperature applications under strenuous environments. A comparison of the elevated temperature surface stability of Rene' 150 alloy and the alloy of the present invention has shown that during 100 hours exposure to Mach 1 air, Rene' 150 alloy at 1135°C (2075°F) lost 1.27-1.65mm (50-65 mils) of metal per specimen side, whereas the alloy of the present invention, in the form shown in Table II, at a higher temperature of 1177°C (2150°F) and a longer exposure time of 150 hours lost only 0.038mm (1.5 mils) per specimen side, i.e. less than about 0.127mm (5 mils) per side according to this invention. In another test, for additional comparison, Rene' 150 alloy at 1135°C (2075°F) in Mach 1 airflow lost 1.016mm (40 mils) per specimen side after 82 hours.

One nickel base alloy considered to have outstanding elevated temperature oxidation resistance is MA754 alloy, identified in Table II. Such alloy is a wrought rather than cast alloy but is included here for further comparison with the oxidation resistance of the present invention. After exposure of a specimen of MA 754 at Mach 1 airflow and 1177°C (2150°F) loss of 0.254mm (10 mils) per specimen side occurred after 140 hours exposure. Confirming the outstanding elevated temperature oxidation resistance of the present invention were tests conducted on specimens from a 1361 kg (3000 pound) heat of the alloy of the present invention. After 170 hours exposure at 1177°C (2150°F) and Mach 1 airflow, a specimen showed a metal loss of only 0.041mm (1.6 mils) per side; after 176 hours at those conditions, a loss of only 0.051mm (2 mils) of metal per side was observed.

Another form of a comparison of this outstanding elevated temperature surface stability, as represented by oxidation resistance, of the present invention with other alloys is shown in the graphical presentation of the drawing. That comparison shows surface loss of a specimen in terms of hours of exposure in high velocity air (HVO) moving at a speed of Mach 1 at 1177°C (2150°C). The Mach 1 oxidation test specimens referred to herein were 5.84mm (0.23") diameter by 88.9mm (3.5") long. Twenty-four specimens were mounted on a round metal plate and tested in a furnace which is heated by aircraft jet fuel. The test specimens were examined about every 24 hours. As can be seen, the present invention provides a cast article with remarkable surface stability.

As was stated above, an important characteristic of the present invention is its improved longitudinal stress rupture strength and improved balance between longitudinal and transverse stress rupture properties along with the outstanding surface stability discussed above. It exhibits, in a DS columnar grain article, the good stress rupture strength of Rene' 150 alloy and outstanding oxidation resistance of the single crystal article of the Rene' N5 composition in Table II above. The following Table IV compares certain stress rupture properties:

**TABLE IV**

| LONGITUDINAL STRESS RUPTURE DATA (uncoated, 0.160 diameter bars) | | | | |
|---|---|---|---|---|
| TEMP °C (°F) | STRESS MPa (ksi) | ALLOY/RUPTURE LIFE (hours) | | |
| | | INVENTION(DS) | RENE' 150(DS) | RENE' N4(a) |
| 982 (1800) | 276 (40) | 40 - 70 | 40 - 70 | 60 |
| 871 (1600) | 552 (80) | 45 - 100 | 50 - 90 | 65 |

| | | | | |
|---|---|---|---|---|
| (a) Single crystal, diffusion aluminide coated. | | | | |

For the alloy of the present invention, the transverse stress rupture strength at 982°C (1800°F) and 221 MPa (32,000 psi)(32 ksi) nominally was in the range of about 80 - 120 hours, as shown in Table V below.

During the evaluation of the present invention, several heat treatments were studied. In one series of heat treatment tests, the alloy associated with the present invention and nominally described in Table II was DS cast into 0.635cm (1/4") thick x 5.08cm (2") wide x 10.16cm (4") long columnar grain slabs from which standard stress rupture specimens were machined after heat treatment of the slabs. In previous evaluations, for example with Rene' 150 alloy columnar grain articles, only partial solutioning was necessary to develop desired properties and full solutioning (90 - 95%) seriously reduced transverse stress rupture properties. However, it was found that the present invention requires substantially full solution heat treatment (at least 90% solutioning of the gamma - gamma prime eutectic and coarse secondary gamma prime with no more than about 4% incipient melting) in order to develop desired properties. In addition to the initial substantially full solutioning, a preferred form of the heat treatment of the present invention includes an additional progressive combination of aging steps: a primary, first aging to improve ductility and transverse stress rupture properties, and two additional aging treatments at temperatures consecutively lower than that of the primary age to further optimize the gamma prime precipitate.

An outline of a series of heat treatments evaluated, along with resulting stress rupture strength, is shown in the following Table V. The heat treatments, identified as A, B, C and D, summarize the heating steps, first with a solution temperature in the range of 1260°C-1279°C (2300-2335°F) for 2 hours. This is followed by a progressive combination and series of aging steps identified in a manner widely used and understood in the metallurgical art. The solution and aging steps were conducted in a non-oxidizing atmosphere: vacuum, argon or helium. Cooling below 649°C (1200°F) conducted between aging steps, need not be conducted in such an atmosphere. Of the heat treatments evaluated, heat treatment D, involving a unique relatively slow cooling step from the first aging to the temperature at which the second aging temperature was to be conducted, resulted in the best combination of properties.

In the heat treatment of the present invention, a substantially full solutioning step is included. This is in contrast with the partial solutioning commonly used with such DS articles made from alloys from Table II such as Rene' 150, certain properties of which are affected detrimentally by a full solution heat treatment. In this invention, solutioning of at least about 90% of the gamma - gamma prime eutectic and coarse secondary gamma prime and with less than about 4%incipient melting is important because the stress rupture life is increased with increased solutioning of the gamma prime eutectic and coarse secondary gamma prime. The following Table VI compares amount of solutioning and stress rupture life for the alloy associated with the present invention.

**TABLE VI**

| Effect of Solutioning on Stress Rupture Life | |
|---|---|
| % Unsolutioned | 982°C (1800°F) Stress Rupture Life |
| 20 | x |
| 10 - 15 | 2x |
| 0 - 5 | 3x |

After solutioning, it is preferred that cooling, for example to a temperature in the range of 1107-1135°C (2025-2075°F) be at a rate of at least 56°C (100°F) per minute. As described in US-A-5100984, more rapid cooling rates have a beneficial effect on properties such as stress rupture strength.

The heat treatment of the present invention is further characterized by a progressive combination of aging stops after solutioning The first or primary age is conducted in a temperature range of 1107-1135°C (2025-2075°F) in a non-oxidizing atmosphere, for example for about 1 - 10 hours, to improve ductility and stress rupture strength of the article. After the first solutioning, it is preferred that cooling, for example to the range of 1066-1093°C (1950-2000°F) be at a rate of about 42°C (75°F) per hour prior to further cooling. A second aging step, at a temperature lower than the first aging, for example in the range of 1066-1093°C (1950-2000°F) for about 4-12 hours, generally about 4-8 hours, enables growth of the gamma prime to improve ductility, As can be seen from the data of Table V, this unique progressive combination of heating steps results in a structure of improved mechanical properties and enables heat treatment of castings having thin walls without detrimental affect on such walls.

After the above aging steps, a final aging step generally is beneficial, for example, in the range of 885-913°C (1625-1675°F) for about 2-10 hours, typically about 4-8 hours.

The heat treatment of the present invention, in connection with the DS cast article utilizing the alloy associated with this invention maximizes longitudinal stress rupture strength while retaining acceptable transverse strength and ductility. This is due, at least in part, to the increased solutioning of the gamma prime at a relatively higher temperature, Introduction of a primary or first aging in the range of 1107-1135°C (2025-2075°F) followed by a relatively slow cool (for example, about 1 hour) to a temperature in the range of 1066-1093°C (1950-2000°F) before further cooling resulted in a further improvement in longitudinal stress rupture life coupled with improved transverse stress rupture properties.

The combination of alloy selection, casting practice, and heat treatment, according to the present invention, enables provision of an improved DS columnar grain article including a thin wall of less than about 0.889mm (0.035 inch) substantially free of cracks. In the form of a gas turbine engine turbine blade, which has a radial centerline, the grain boundaries and primary dendritic orientation is approximately straight and parallel. In addition, it is preferred in such an article, and is capable through this invention, that any emergent grain from the airfoil of such a blade intersect the airfoil leading edge or trailing edge at an angle no greater than 15° with the edge and that all other grain boundaries and primary dendrites are within 15° of the radial centerline.

As a result of evaluations of the type described above, it was recognized that the heat treatment of the present invention can be used with a particular alloy range. A specific alloy range is particularly unique in the combination with the heat treatment. The following Table VII identifies such useful and specific alloy range.

**Table VII**

| ALLOY COMPOSITION FORMS Wt%, balance Ni and incidental impurities | | | |
|---|---|---|---|
| ELEMENTS | RANGES | | |
| | BROAD | PREFERRED | SPECIFIC |
| C | 0.1-0.15 | 0.1-0.15 | 0.1-0.14 |
| Hf | 0.3-2 | 1-2 | 1.2-1.7 |
| Co | 11-14 | 11-13 | 11.7-12.3 |
| Ta | 5-9 | 6-7 | 6.2-6.5 |
| V | no more than 1 | less than 1 | 0-0.1 |
| Zr | less than .05 | 0-.03 | 0-0.03 |
| Cr | 5-10 | 6-7 | 6.6-7 |
| Mo | 0.5-3 | 1-2 | 1.3-1.7 |
| W | 4-7 | 4.5-5.5 | 4.7-5.1 |
| Ti | no more than 1 | less than 1 | 0-0.02 |
| Al | 5-7 | 5.5-6.5 | 6-6.3 |
| Re | 1.5-4 | 2.5-3.5 | 2.6-3 |
| B | .005-.03 | .01-.02 | .01-.02 |
| Cb | 0-1.5 | 0-0.5 | 0-0.1 |
| Y | 0-0.5 | 0-0.5 | 0-0.2 |

This invention has been described in connection with specific examples and embodiments. However, it will be understood by those skilled in the metallurgical arts involved that the invention is capable of a variety of other forms and embodiments within the scope of the appended claims.

## Claims

1. A nickel base superalloy consisting of in weight percent 0.12% carbon, 1.5% hafnium, 12% cobalt, 6.35% tantalum, 6.8% chromium, 1.5% molybdenum, 4.9% tungsten, 6.15% aluminum, 2.8% rhenium, 0.015% boron, the substantial absence of zirconium, the substantial absence of titanium, the substantial absence of vanadium and the balance nickel and incidental impurities.

2. An article of the alloy of Claim 1 having an internal cavity within an outside article surface, the cavity including an integral cast wall, substantially free of cracks, and a wall thickness of less than about 0.889mm (0.035 inch).

3. The article of Claim 2 in which the internal cavity is separated from the outside surface by an article wall across a thickness of less than about 0.889mm (0.035 inch).

4. The cast article of Claim 2 in the form of a turbine blading member having a radial centerline and including an airfoil having a leading edge and a trailing edge in which :
grain boundaries and primary dendritic orientation is approximately straight and parallel; and
any emergent grain which intersects the airfoil leading or trailing edge forms an angle no greater than 15° with the edge, and all other grain boundaries and primary dendrites are within 15° of the radial centerline.

5. The article of Claim 1 wherein the article is a gas turbine engine airfoil.

6. A method of heat treating a cast nickel base alloy article made of an alloy consisting of, in weight percent, 0.1-0.15 C, 0.3-2 Hf, 11-14 Co, 5-9 Ta, less than 0.05 Zr, no more than 1 of V, no more than 1 of Ti, 5-10 Cr, 0.5-3 Mo, 4-7 W, 5-7 Al, 1.5-4 Re, 0.005-0.03 B, up to 1.5 Nb, up to 0.5 Y and the balance Ni and incidental impurities comprising the steps of :
(a) heating at a solutioning temperature in a non-oxidizing atmosphere for a time sufficient to solution at least 90% of the gamma-gamma prime eutectic and coarse secondary gamma prime and so that there is no more than about 4% incipient melting, and then cooling in the atmosphere to a temperature in the range of 1107-1135°C (2025°-2075°F);
(b) heating at a first aging temperature in the range of 1107-1135°C (2025°-2075°F) in a non-oxidizing atmosphere for 1-10 hours and then cooling in the atmosphere to a temperature in the range of 1066-1093°C (1950°-2000°F); and
(c) heating at a second aging temperature lower than the first aging temperature in the range of 1066-1093°C (1950°-2000°F) for 4-12 hours.

7. The method of Claim 6 in which the solutioning temperature is in the range of 1246-1293°C (2275°-2360°F) and the heating time is at least about 30 minutes.

8. The method of Claim 6 or Claim 7 including a third aging step of :
(d) heating at a temperature range of 885-913°C (1625°-1675°F) for 2-10 hours.

9. A method of making a cast columnar grain nickel base superalloy article of outstanding elevated temperature oxidation resistance, the article having an internal cavity including an integral cast wall of a wall thickness of less than about 0.889mm (0.035 inch) comprising the steps of :
(a) precision casting the article from an alloy consisting of, in weight percent, 0.1-0.15C, 0.3-2 Hf, 11-14 Co, 5-9 Ta, less than 0.05 Zr and no more than 1 of each of V and Ti, 5-10 Cr, 0.5-3 Mo, 4-7 W, 5-7 Al, 1.5-4 Re, 0.005-0.03 B, up to 1.5 Nb, up to 0.5 Y and the balance Ni and incidental impurities, with the cast wall integral with the casting by columnar multigrain directional solidification casting; and
(b) heat treating the cast article in accordance with Claim 6.

10. The method for making a cast columnar grain nickel base superalloy gas turbine engine turbine blading member of outstanding elevated temperature oxidation resistance, the article having at least one internal cavity including an integral cast wall of a wall thickness less than about 0.889mm (0.035 inch) comprising the steps of :
(a) providing a superalloy consisting of, in weight percent, 0.1-0.14 C, 1.2-1.7 Hf, 11.7-12.3 Co, 6.2-6.5 Ta, up to 0.1 V, up to 0.03 Zr, 6.6-7 Cr, 1.3-1.7 Mo, 4.7-5.1 W, no more than 0.02 Ti, 6-6.3 Al, 2.6-3 Re, 0.01-0.02 B, up to 0.1 Nb, up to 0.2 Y, and the balance Ni and incidental impurities;
(b) precision casting said superalloy to provide an article having at least one internal cavity including an integral cast wall of a wall thickness of less than about 0.889mm (0.035 inch); and
(c) heat treating said cast article in accordance with Claim 7.

## Patentansprüche

1. Superlegierung auf Nickelbasis, bestehend aus, in Gew.-%, 0,12% Kohlenstoff, 1,5% Hafnium, 12% Cobalt, 6,35% Tantal, 6,8% Chrom, 1,5% Molybdän, 4,9% Wolfram, 6,15% Aluminium, 2,8% Rhenium, 0,015% Brom, wobei Zirkonium, Titan und Vanadium im wesentlichen abwesend und der Rest Nickel und übliche Verunreinigungen sind.

2. Gegenstand aus der Legierung nach Anspruch 1 mit einem inneren Hohlraum innerhalb einer äußeren Gegenstandsoberfläche, wobei der Hohlraum eine integral gegossene Wand einschließt, die im wesentlichen frei von Rissen ist und eine Dicke von weniger als etwa 0,889 mm (0,035 inch) hat.

3. Gegenstand nach Anspruch 2, worin der innere Hohlraum von der äußeren Oberfläche durch eine Gegenstandswand über eine Dicke von weniger als etwa 0,889 mm (0,035 inch) getrennt ist.

4. Gußteil nach Anspruch 2 in Form einer Turbinenschaufel mit einer radialen Mittellinie und mit einem Flügel mit einer Vorderkante und einer rückwärtigen Kante, bei dem:
die Korngrenzenorientierung und die Orientierung der primären Dentriten etwa gerade und parallel ist und
jedes austretende Korn, das die Vorder- oder rückwärtige Kante des Flügels schneidet, mit dieser Kante einen Winkel von nicht mehr als 15° bildet und alle anderen Korngrenzen und primären Dentriten innerhalb von 15° der radialen Mittellinie liegen.

5. Gegenstand nach Anspruch 1, der ein Flügel einer Gasturbine ist.

6. Verfahren zum Wärmebehandeln eines Gußteiles aus einer Nickellegierung, hergestellt aus einer Legierung, bestehend aus, in Gew.-%, 0,1-0,15 C, 0,3-2 Hf, 11-14 Co, 5-9 Ta, weniger als 0,05 Zr, nicht mehr als 1 V, nicht mehr als 1 Ti, 5-10 Cr, 0,5-3 Mo, 4-7 W, 5-7 Al, 1,5-4 Re, 0,005-0,03 B, bis zu 1,5 Nb, bis zu 0,5 Y, der Rest sind Nickel und übliche Verunreinigungen, umfassend die Stufen:
(a) Erhitzen bei einer Lösungstemperatur in einer nicht oxidierenden Atmosphäre für eine Zeit, die zur Lösung von mindestens 90% des Gamma-Gamma'-Eutektikums und grober sekundärer Gamma' genügt, und daß nicht mehr als etwa 4% beginnendes Schmelzen auftritt und dann Abkühlen in der Atmosphäre auf eine Temperatur im Bereich von 1107-1135°C (2025°-2075°F);
(b) Erhitzen auf eine erste Alterungstemperatur im Bereich von 1107-1135°C (2025°-2075°F) in einer nicht oxidierenden Atmosphäre für 1-10 Stunden und dann Abkühlen in der Atmosphäre auf eine Temperatur im Bereich von 1066 bis 1093°C (1950°-2000°F) und
(c) Erhitzen auf eine zweite Alterungstemperatur, die geringer als die erste Alterungstemperatur ist und im Bereich von 1066-1093°C (1950°-2000°F) liegt, für 4-12 Stunden.

7. Verfahren nach Anspruch 6, bei dem die Lösungstemperatur im Bereich von 1246-1293°C (2275°-2360°F) liegt, und die Erhitzungszeit mindestens etwa 30 Minuten beträgt.

8. Verfahren nach Anspruch 6 oder 7, das eine dritte Alterungsstufe des
(d) Erhitzens auf eine Temperatur von 885-913°C (1625°-1675°F) für 2-10 Stunden einschließt.

9. Verfahren zum Herstellen eines Gußteiles mit stengelförmigen Körnern aus Superlegierung auf Nickelbasis mit hervorragender Oxidationsbeständigkeit bei erhöhter Temperatur, wobei das Teil einen inneren Hohlraum mit einer integralen Gußwand einer Dicke von weniger als etwa 0,889 mm (0,035 inch) einschließt, umfassend die Stufen:
(a) Präzisionsgießen des Teiles aus einer Legierung, bestehend aus, in Gew.-%, 0,1-0,15 C, 0,3-2 Hf, 11-14 Co, 5-9 Ta, weniger als 0,05 Zr, nicht mehr als 1 V, nicht mehr als 1 Ti, 5-10 Cr, 0,5-3 Mo, 4-7 W, 5-7 Al, 1,5-4 Re, 0,005-0,03 B, bis zu 1,5 Nb, bis zu 0,5 Y, der Rest sind Nickel und übliche Verunreinigungen, wobei die Gußwand integral mit dem durch gerichtete Erstarrung erhaltenen Gußkörper mit einer Vielzahl stengelförmiger Körner ist und
(b) Wärmebehandeln des Gußteiles gemäß Anspruch 6.

10. Verfahren zum Herstellen einer gegossenen Gasturbinenschaufel mit Stengelkorn aus Superlegierung auf Nickelbasis mit ausgezeichneter Oxidationsbeständigkeit bei erhöhter Temperatur, wobei der Gegenstand mindestens einen inneren Hohlraum aufweist, der eine integrale Gußwand einer Dicke von weniger als etwa 0,889 mm (0,035 inch) einschließt, umfassend die Stufen:
(a) Schaffen einer Superlegierung, bestehend aus, in Gew.-%, 0,1-0,14 C, 1,2-1,7 Hf, 11,7-12,3 Co, 6,2-6,5 Ta, bis zu 0,1 V, bis zu 0,03 Zr, 6,6-7 Cr, 1,3-1,7 Mo, 4,7-5,1 W, nicht mehr als 0,02 Ti, 6-6,3 Al, 2,6-3 Re, 0,01-0,02 B, bis zu 0,1 Nb, bis zu 0,2 Y und der Rest sind Ni und übliche Verunreinigungen;
(b) Präzisionsgießen der Superlegierung zur Schaffung eines Gegenstandes mit mindestens einem inneren Hohlraum, der eine integrale Gußwand einer Dicke von weniger als etwa 0,889 mm (0,035 inch) einschließt und
(c) Wärmebehandeln des Gußteiles gemäß Anspruch 7.

## Revendications

1. Superalliage à base de nickel consistant, en pourcentage en poids, en 0,12% de carbone, 1,5% de hafnium, 12% de cobalt, 6,35% de tantale, 6,8% de chrome, 1,5% de molybdène, 4,9 % de tungstène, 6,15 % d'aluminium, 2,8% de rhénium, 0,015% de bore, une absence substantielle de zirconium, une absence substantielle de titane, une absence substantielle de vanadium, le complément étant du nickel et des impuretés accidentelles.

2. Article en alliage selon la revendication 1 comportant une cavité interne dans la surface extérieure de l'article, la cavité comprenant une paroi venue de moulage d'une seule pièrce, sensiblement exempte de fissures, et ayant une épaisseur inférieure à environ 0,889mm (0,035 inch).

3. Article selon la revendication 2, dans lequel la cavité interne est séparée de la surface extérieure par l'épaisseur de l'article, inférieure à environ 0,889mm (0,035 inch).

4. Article moulé selon la revendication 2 sous la forme d'un élément d'aubage de turbine ayant un axe radial et comprenant une partie aérodynamique comprenant un bord d'attaque et un bord de fuite, dans lequel
les joints des grains et l'orientation dendritique principale sont approximativement rectilignes et parallèles; et
tout grain émergent qui intersecte le bord d'attaque ou le bord de fuite forme avec le bord un angle qui n'est pas supérieur à 15 degrés, et tous les autres joints de grains et dendrites principales se trouvent à l'intérieur d'un angle de 15 degrés par rapport à l'axe radial.

5. Article selon la revendication 1, dans lequel l'article est un profil aérodynamique d'un turbomoteur.

6. Procédé de traitement thermique d'un article moulé en alliage à base de nickel consistant, en pourcentage en poids, en 0,1-0,15 de C, 0,3-2 de Hf, 11-14 de Co, 5-9 de Ta, moins de 0,05 de Zr, pas plus qu'environ 1 de V, pas plus qu'environ 1 de Ti, 5-10 de Cr, 0,5-3 de Mo, 4-7 de W, 5-7 de Al, 1,5-4 de Re, 0,005-0,03 de B, jusqu'à 1,5 de Nb, jusqu'à 0,5 de Y, le complément étant du Ni et des impuretés accidentelles, ce procédé comprenant les étapes consistant :
(a) à chauffer à une température de mise en solution dans une atmosphère non-oxydante pendant un temps suffisant pour mettre en solution au moins 90% de la phase eutectique gamma-gamma prime et de la phase gamma secondaire à grains grossiers et de façon qu'il n'y ait pas plus qu'environ 4% de fusion commençante, et à refroidir ensuite dans l'atmosphère jusqu'à une température comprise dans la plage de 1107-1135°C (2025-2075°F);
(b) à chauffer à une première température de vieillissement comprise dans la plage de 1107-1135°C (2025-2075°F) dans une atmosphère non oxydante pendant 1-10 heures, et à refroidir ensuite dans l'atmosphère juqu'à une température comprise dans la plage de 1066-1093°C (1950-2000°F); et
(c) à chauffer à une seconde température de vieillissement inférieure à la première température de vieillissement et comprise dans la plage de 1066-1093°C (1950-2000°F) pendant 4-12 heures.

7. Procédé selon la revendication 6 dans lequel la température de mise en solution est comprise dans la plage de 1246-1293°C (2275-2360°F) et le temps de chauffage est d'au moins environ 30 minutes.

8. Procédé selon la revendication 6 ou la revendication 7 comprenant une troisième étape de vieillissement consistant :
(d) à chauffer à une température comprise dans la plage de 885-913°C (1625-1675°F) pendant 2-10 heures.

9. Procédé pour fabriquer un article moulé en superalliage à base de nickel à grains colonnaires présentant une très grande résistance à l'oxydation aux température élevées, cet article comportant une cavité interne comprenant une paroi venue de moulage d'une seule pièce et ayant une épaisseur inférieure à environ 0,889mm (0.035 inch), comprenant les étapes consistant :
(a) à effectuer un moulage de précision de l'article à partir d'un alliage consistant, en pourcentage en poids, en 0,1-0,15 de C, 0,3-2 de Hf, 11-14 de Co, 5-9 de Ta, moins de 0,05 de Zr et pas plus de 1 de chacun deV et de Ti, 5-10 de Cr, 0,5-3 de Mo, 4-7 de W, 5-7 de Al, 1,5-4 de Re, 0,005-0,03 de B, jusqu'à 1,5 de Nb, jusqu'à 0,5 de Y, le complément étant Ni et des impuretés accidentelles, la paroi moulée faisant corps avec la pièce moulée par suite du moulage avec solidification directionnelle multigrains colonnaires;
(b) à traiter thermiquement l'article moulé selon la revendication 6.

10. Procédé pour fabriquer un élément moulé d'aubage de turbine de turbomoteur en superalliage à base de nickel à grains colonnaires présentant une très grande résistance à l'oxydation aux températures élevées, cet article comportant au moins une cavité interne comprenant une paroi venue de moulage d'une seule pièce, d'une épaisseur inférieure à environ 0,889mm (0,035 inch), ce procédé comprenant les étapes consistant :
(a) à préparer un superalliage consistant , en pourcentage en poids, en 0,1-0,14 de C, 1,2-1,7 de Hf, 11,7-12,3 de Co, 6,2-6,5 de Ta, jusqu'à 0,1 de V, jusqu'à 0,03 de Zr, 6,6-7 de Cr, 1,3-1,7 de Mo, 4,7-5,1 de W, pas plus de 0,02 de Ti, 6-6,3 de Al, 2,6-3 de Re, 0,01-0,02 de B, jusqu'à 0,1 de Nb, jusqu'à 0,2 de Y, le complément étant du Ni et des impuretés accidentelles;
(b) à effectuer un moulage de précision dudit superalliage pour obtenir un article ayant au moins une cavité interne comprenant une paroi venue de moulage d'une seule pièce, d'une épaisseur de moins de 0,889mm (0,035 inch); et
(c) à traiter thermiquement ledit article moulé selon la revendication 7.
